

Sept. 26, 1933.

J. HARRINGTON

**1,927,830**

## MEANS AND METHOD OF HEAT TREATING CERAMIC MATERIALS

Filed Oct. 6, 1930

2 Sheets-Sheet 1



Inventor:  
Joseph Harrington  
By Cheever, Cox & Moore

Atty.

Sept. 26, 1933.

J. HARRINGTON

1,927,830

## MEANS AND METHOD OF HEAT TREATING CERAMIC MATERIALS

Filed Oct. 6, 1930

2 Sheets-Sheet 2



Inventor:  
Joseph Harrington  
By Cheever, Cox & Moore

## UNITED STATES PATENT OFFICE

1,927,830

MEANS AND METHOD OF HEAT TREATING  
CERAMIC MATERIALSJoseph Harrington, Riverside, Ill., assignor to  
Joseph Harrington Company, Harvey, Ill., a  
corporation of Illinois

Application October 6, 1930. Serial No. 486,573

10 Claims. (Cl. 25—145)

My invention relates generally to means for and methods of heat treating ceramic materials, and more particularly to apparatus and methods for heat treating such materials as brick within a kiln chamber.

In burning ware such as brick and other clay products, a certain period of the burning is required for burning out or oxidizing the carbon in the clay. During this period it is necessary to have an excess of oxygen within the kiln chamber in order to obtain the proper oxidizing effects. After this period of oxidation has continued for a predetermined period of time, it is desirable to produce a surface color or what is commonly known in the trade as "flashing" to the ware and this is accomplished by subjecting the ware within the kiln to a reducing atmosphere. That is to say, the atmosphere within the kiln is such as to reduce or de-oxidize certain metallic or other oxides on the surface of the ware to produce certain colors or textures on said surface.

It is one of the primary objects of my present invention to provide improved methods and means whereby the above mentioned oxidizing and reducing atmospheres within the kiln chamber may be obtained.

More specifically, it is an object of my invention to provide a reducing atmosphere within a kiln chamber by burning bituminous fuel in such a manner as to supply a deficiency of oxygen so that incomplete combustion of the carbon within the fuel takes place, thereby producing carbon monoxide.

Still more specifically, my invention contemplates the production of a reducing atmosphere within a kiln chamber by supplying an excess of carbon for the oxygen present within a fuel bed, thereby producing the same effect as incomplete combustion. In other words, producing carbon monoxide for use in the kiln chamber.

Still another object of my invention is to control atmospheric conditions within a kiln chamber by varying the thickness of the fuel bed, the variation in the fuel bed thickness serving to control the amount of oxygen within the kiln chamber.

My invention is not limited to the production of oxidizing conditions within a kiln chamber by varying the thickness of a fuel bed, but contemplates other means and methods whereby the combustion of a bed of fuel, such as bituminous fuel, may be controlled so as to produce proper oxidizing and reducing conditions within the kiln.

A still further object of my invention is to produce oxidizing and reducing conditions within a kiln chamber, as above set forth, by introducing heated gases from an external source under pressure, above atmospheric pressure where-  
by to prevent the leakage of cold air through the cracks and crevices of the kiln.

In addition to the above mentioned objects and advantages, my invention contemplates the provision of a kiln in which hot gases under a pressure above atmospheric pressure, may be introduced in the central lower portion of the kiln chamber, the ware within the chamber providing a central passage for directing the heated gases to the upper portion of the chamber from which point said gases pass downwardly through the ware so as to effect the uniform burning thereof, said gases being drawn off through suitable passageways connected with the lower portion of the kiln.

The foregoing and numerous other objects and advantages will be more apparent from the following detailed description, when considered in connection with the accompanying drawings, wherein:

Figure 1 is a vertical sectional view of a device whereby my improved method of heat treating ceramic materials may be effectively practiced;

Figure 2 is an enlarged semi-diagrammatic disclosure in section of an automatic furnace or stoker, said device being provided with a fuel bed capable of producing oxidizing conditions within the kiln chamber; and

Figure 3 is a view similar to Figure 2, disclosing a fuel bed of increased thickness whereby reducing atmospheric conditions within the kiln chamber may be maintained.

Referring now to the drawings more in detail wherein like numerals have been employed to designate similar parts throughout the various figures, it will be seen that one embodiment of my invention resides in the provision of a dome shaped kiln which I have designated generally by the numeral 10. This kiln may be of any suitable refractory material and is provided with a suitable floor 12 having a plurality of apertures 14. These apertures 14 communicate with a common egress chamber or passage 16 which passage in turn communicates with a central annular passage 18. Gases from this passage 18 may be withdrawn through a suitable horizontal passage 20, Figure 1. Heated gases are introduced within the chamber 22 of the kiln 10 from a conduit or passage 24 which opens into

the central lower portion of the chamber as clearly shown in Figure 1. This passage 24 communicates at its opposite extremity with the discharge side of a combustion chamber 26 provided within 5 a suitable furnace or stoker which I have designated generally by the numeral 28.

This stoker or furnace 28 is positioned externally of the kiln chamber as clearly shown in Figure 1 and I prefer to have the furnace positioned below the kiln chamber so as to facilitate 10 the passage of the heated gases from the stoker to said chamber. This stoker may be of the type described and claimed in detail in my copending application, Serial Number 340,924, filed February 18, 1929, although my invention is not limited 15 to any particular furnace or stoker construction. The stoker 28 includes a suitable fuel hopper 30 and fuel 32 from this hopper is directed to a reciprocable fuel receiving plate 34. Reciprocation 20 is imparted to this plate 34 in any suitable manner, as for example, through the agency of an oscillatory bar 36 which is operatively connected with a depending arm 38 of the plate by means of a horizontal link 40 interposed between the 25 arm 38 and the free extremity of a lever arm 42. The plate 34 is supported by rollers 44 which are in turn supported by suitable guides 46, Figures 2 and 3. The left or rearward extremity of the plate 34 is connected with a grate section 48 and this section rests upon a stationary grate section 50. The rearward portion of this grate section 50 is formed with an upwardly projecting portion or hump 52 which serves to control the thickness of 30 the fuel bed within the combustion chamber 26.

The rearward or left extremity of this grate section 50 rests upon a receptacle grate section 54 which is also provided with an upwardly projecting portion or hump 56. Reciprocation is 35 imparted to this section 54 by means of an elongated link 58 which is detachably connected at its forward extremity with a pin 60 mounted at the free extremity of the arm 42. A notch 60a, Figure 3, is provided in the link 58 and when the link occupies the position shown in Figure 2, this 40 notch 60a receives the pin 60, thereby coupling the arm 42 with the grate 54. However, when the link 58 is elevated by manipulating a suitable control lever 62, the link occupies the position shown in Figure 3, thereby disconnecting the oscillatory arm 42 from the grate 54. In other words, the grate 54 is reciprocable when the link 58 is connected to the pin 60 and is stationary 45 when said link is disconnected from said pin.

The grate 54 rests upon a rear stationary grate section 64 and this section serves to direct ashes to the ash pit 66. A suitable partition 67 serves to separate the horizontal portion of the ash pit 66 from a chamber 68. This chamber 68 is adapted to receive air for draft purposes from 50 an adjoining chamber 70, Figure 1.

This chamber 70 receives air under pressure from a suitable air pump 72, Figure 1. In this connection it should be noted that the chamber 70 is enclosed by a sealing wall 74. The air pressure within the chamber is maintained at 55 slightly greater pressure than the pressure within the stoker and hence proper draft conditions upwardly through the fuel bed supported by the stoker grates is constantly maintained. The advantages resulting from the provision of the sealing wall 74 will be apparent when it is understood that it is very difficult to construct a furnace or stoker which is free from leaks at all 60 points. Even the porous condition of the material used in the construction of the furnace is often

sufficient to establish a certain amount of leakage. Hence, by subjecting the entire stoker unit to an increased external pressure, leakage through the stoker walls is positively prevented and I am able to supply heated gases under pressure above atmospheric pressure to the kiln chamber 22. 80

In Figure 2 I have shown a fuel bed designated by the letter A and this fuel bed is maintained within the combustion chamber when the grate 48 with its associated fuel receiving plate 34 and the grate 54 are reciprocated. The reciprocation of these grates causes a fuel bed of uniform moderate thickness to be built up and advanced through the combustion chamber. This fuel bed 85 A is the type of bed which is employed to produce an oxidizing atmosphere within the kiln chamber 22. It should be noted that I contemplate piling the ware or brick 76 within the kiln chamber so as to present a central flue or passage 90 78. The lower reduced portion of this passage or flue 78 communicates with the passageway 24 extending from the combustion chamber and the upper extremity of the passage 95 78 terminates at the upper central portion of the kiln chamber. Thus, hot gases introduced at the bottom of the kiln pass upwardly through the flue 78 and are then uniformly dispersed within the kiln chamber so as to effect the uniform diffusion of heat to all parts of the kiln 100 chamber. 105

In order to obtain a clear understanding of my improved means and method for heat treating the ware, it is necessary to review in a general way the chemical reactions which take place 110 in the fuel bed insofar as they apply to the formation of carbon monoxide (CO) and carbon dioxide (CO<sub>2</sub>). Referring first to Figure 2 wherein I have disclosed the fuel bed A which is employed to effect the oxidation within the kiln chamber, it will be seen that air for combustion passes upwardly through the grate surfaces, and the oxygen of this air first encounters the fixed carbon or coke at the lower incandescent surface of the fuel bed. It then combines with this carbon to form carbon dioxide (CO<sub>2</sub>), but the fuel bed is sufficiently thick and contains voids or channels of sufficient amount so that combustion is complete and carbon dioxide (CO<sub>2</sub>) escapes through these passageways or 115 voids to the upper surface of the fuel bed without further contact with the carbon. Thus, the gas emerging from such a fuel bed as the bed 120 A contains a high percentage of carbon dioxide (CO<sub>2</sub>) and little or no carbon monoxide (CO). 125 As a matter of fact, there is practically universally an excess of oxygen which finds its way through the voids in the fuel bed, and the resultant gases carry substantially from 2 to 130 8 percent of free oxygen. This gas which emerges from the fuel bed A is called an oxidizing 135 gas or atmosphere, and it is this free oxygen at high temperatures that burns out the carbon contained in the clay of the ware, wherein the temperature of the ware reaches a certain definite amount. Thus, when the stoker 28 is operating so as to present the fuel bed A, I am able 140 to produce an oxidizing atmosphere within the kiln chamber so as to effect burning out of the carbon in the clay of the ware. This burning process is continued for a predetermined time 145 until the ware is in condition to be "flashed", that is, to be subjected to a reducing atmosphere for the purpose of producing a desired surface color. 150

This reducing atmosphere may be produced in various ways and for the purpose of illustrating one practical method, I have shown means whereby the thickness of the fuel bed may be increased. 5 When it is desired to change the oxidizing atmosphere within the kiln chamber to a reducing atmosphere, it is only necessary to manually shift the control lever 62 downwardly to the position shown in Figure 3. This causes the uncoupling 10 of the grate 54 from the actuating arm 42, as clearly shown in Figure 3, and under such conditions the only movable grate section is the section 48 and its companion fuel receiving plate 34. Under such conditions the distance between the 15 pushing face of the grate 48 and the rear of the stoker is so great that the friction of the fuel thereon will act as a dam or check to the flow of the fuel and hence will necessarily effect the piling up of the fuel to a considerable thickness 20 within the kiln chamber. In other words, the thickness of the fuel bed will be materially increased and I have designated this fuel bed of increased thickness by A<sup>1</sup>, Figure 3. By having this fuel bed of increased thickness, I obtain a 25 different chemical reaction within the fuel bed which serves to produce a reducing atmosphere within the kiln chamber. Thus, in the fuel bed A<sup>1</sup> there is a thicker layer of incandescent coke on the supporting grate and air enters the fuel 30 bed from below, as previously described, and the oxygen thereof combines with the bottom layer of carbon to form carbon dioxide (CO<sub>2</sub>) as also stated above. However, the increased thickness 35 of the incandescent coke prevents a large quantity of carbon which at these temperatures will break down the carbon dioxide (CO<sub>2</sub>) and cause it to become carbon monoxide (CO). There being no further air for combustion available at this point, the carbon monoxide (CO) will emerge 40 from the surface of the fuel bed and presents what may be referred to as a reducing atmosphere within the kiln chamber. The stoker 28 may be continuously operated under the thick fuel bed 45 conditions so as to cause the desired degree of "flashing". It should be remembered that during this entire operation the pressure within the kiln chamber is above atmospheric pressure so as to maintain constant uniform atmospheric conditions within the chamber during this reducing 50 process. Gases from the kiln chamber are continuously withdrawn from the bottom thereof and may be conducted to a second kiln (not shown) and subjected to ware therein, if so desired. Certain kinds of face brick can be permanently colored if allowed to cool several hundred degrees 55 in a reducing atmosphere, and my invention enables this method to be effectively practiced. In other words, the fuel bed conditions within the stoker may be continuously maintained while the 60 kiln is cooling and during this entire time the pressure within the kiln is above atmospheric pressure. Placing the kiln and connecting passages under a pressure above atmospheric is essential because in the conventional operation of 65 a kiln there will be enough infiltration into the kiln chamber through the cracks and other voids in the brickwork to provide all the oxygen needed to offset the reducing atmosphere produced in the furnace. It is essential, therefore, that the 70 kiln be kept under pressure to maintain reducing conditions within the chamber.

From the foregoing description it will be apparent that my invention provides improved means and methods whereby atmospheric conditions within a kiln chamber may be very effec-

tively controlled. More specifically, it might be stated that my invention provides a new and improved method of burning fuel, such as bituminous products, at a point externally of a kiln chamber and controlling the combustion of said fuel so as to present oxidizing or reducing conditions within the kiln chamber. By employing the type of stoker shown in the drawings I obtain smokeless combustion, thereby positively preventing the introduction of smoke within the kiln chamber. By having the stoker positioned at a point spaced from the kiln chamber, I am able to employ all of the space within the kiln chamber for ware to be burned. In fact, the only portion of the kiln which is not taken up by the ware is that portion immediately above the passage or flue 24 and this passage must be present in order to effect the delivery of the heated gases to the upper portion of the kiln chamber. The kiln and its associated parts is very practical in construction and may be very economically manufactured. In fact, my invention presents a decided divergence from the conventional methods of heat treating ceramic materials, such as clay products, and practical tests have conclusively shown that by employing my invention ceramic materials may be heat treated with greater economy and the time necessary for heat treatment materially reduced.

Having thus described my invention, what I claim as new and desire to secure by Letters Patent is:

1. In heat treating apparatus of the class described, a kiln chamber for receiving a supply of ware to be heat treated, an external furnace for supplying heated gases under pressure in excess of atmospheric pressure, means for conducting said heated gases into said kiln chamber, whereby the pressure of the gases in said kiln chamber will be maintained above atmospheric pressure, and means for varying the thickness of the fuel bed within said furnace to control the oxidizing and reducing actions within the kiln chamber.

2. In combination with the chamber of a kiln, a furnace for supplying heated gases, a flue connecting said furnace with the kiln chamber, a casing enclosing said furnace, means for supplying air within said enclosure to maintain pressure surrounding the furnace greater than pressure within the furnace, and means for varying the thickness of the fuel bed in the furnace to control the oxidizing and reducing actions of the gases supplied thereby to the kiln chamber.

3. In heat treating apparatus of the class described, a closed kiln having a chamber for receiving ware to be treated, means for supplying heated gases under pressure in excess of the atmospheric pressure surrounding the kiln, means for conducting said heated gases to the lower central portion of the kiln, and means for withdrawing gases from the lower portion of said kiln.

4. In combination with the chamber of a kiln, a furnace for supplying heated gases including a plurality of relatively reciprocable grate sections within a combustion chamber, a flue connecting said furnace with the kiln chamber, and control means for regulating the relative reciprocation of the grate sections to enable the production of oxidizing and reducing gases for said kiln chamber.

5. In combination with the chamber of a kiln, a furnace for supplying heated gases including a plurality of relatively reciprocable grate sections within a combustion chamber, a flue connecting said furnace with the kiln chamber, and

means for arresting the movement of at least one of said reciprocable grate sections whereby to cause a building up of the fuel within the combustion chamber for the production of reducing gases.

5 6. In heat treating apparatus of the class described, a kiln chamber for receiving a supply of ware to be treated, a furnace for supplying heated gases to said kiln chamber, said furnace including a combustion chamber and means for progressively feeding a bed of fuel therethrough, and means for controlling the movement of the fuel bed through said combustion chamber in accordance with the oxidizing and reducing requirements within the kiln chamber.

10 7. In heat treating apparatus of the class described, a kiln chamber for receiving a supply of material to be treated, means for supplying heated gases to said kiln chamber including a fuel combustion chamber, means to burn fuel in said combustion chamber, and means to regulate the combustion of the fuel in accordance with the oxidizing and reducing requirements of the kiln chamber.

15

8. In heat treating apparatus of the class described, a kiln chamber for receiving material to be treated, means to supply the products of fuel combustion to said chamber and means to regulate the combustion of the fuel in accordance with the oxidizing and reducing requirements within the kiln chamber.

9. The method of heat treating ceramic material, which consists in burning fuel and applying products of combustion to the material being treated while regulating the combustion of the fuel in accordance with the oxidizing and reducing effect required by the heat treatment.

10. The method of heat treating ceramic material, which consists in first oxidizing the material by exposing it to the products of fuel combustion properly regulated to provide oxidizing gases and then exposing the material to be treated to a reducing atmosphere comprising the products of fuel combustion properly regulated to produce reducing gases.

JOSEPH HARRINGTON.

100

30

105

35

110

40

115

45

120

50

125

55

130

60

135

65

140

70

145

75

150

80

85

90

95

105

110

115

120

125

130

135

140

145

150